

Jan. 3, 1939.

W. P. ZABEL

2,142,865

METHOD OF MANUFACTURING FILAMENTS

Filed March 24, 1937

Fig. 1.



Fig. 2.



Fig. 3.



Fig. 4.



Fig. 5.



Fig. 6.



Fig. 7.

OPERATED IN A  
LAMP



Inventor:  
William P. Zabel,  
by Harry E. Benham  
His Attorney.

## UNITED STATES PATENT OFFICE

2,142,865

## METHOD OF MANUFACTURING FILAMENTS

William P. Zabel, Cleveland Heights, Ohio, assignor to General Electric Company, a corporation of New York

Application March 24, 1937, Serial No. 132,763

9 Claims. (Cl. 176—40)

My invention relates to filaments for electric incandescent lamps and more particularly to a process of forming and treating multiple coil filaments preferably of the double (coiled coil) and the triple (coiled coiled-coil) helical type.

One of the objects of my invention is to produce double and triple helical filaments of greater uniformity. Heretofore, the filaments varied somewhat in length and were often distorted. In both cases the direct cause of the defect could not be traced to any particular part of the manufacturing process, largely because the defect was likely to appear in any of the manufacturing steps or even after the filament was operated in a lamp. The defects were believed to be principally the result of changes caused by the relieving of internal strains within the filament, which were produced therein by the particular coiling method used and were not properly relieved by the heat treatment. In some cases the coiling operation alone caused immediate distortion of the filament coils. My process obviates these disadvantages by providing a more satisfactory coiling method and also a heat treating method for relieving the strains produced in the wire by the said coiling method.

Conventional coiling methods heretofore employed have usually consisted in coiling the filament wire on a mandrel of sufficient length to be spooled, coiling the mandrel and filament coiled thereon about a second mandrel and, if the filament was to be of triple helical form, coiling both mandrels and twice coiled filament thereon about a third mandrel. With this method even the twice or thrice coiled filament wire, as the case may be, was coiled in a considerable length which was heat treated and then severed with all mandrels remaining in the filament coils. The mandrels were finally removed by dissolving in an acid.

The conventional method of coiling is objectionable because of the length of the coiling operation since local strains are produced in the filament by variations in the coiling tension which gradually build up until relieved by the twisting of both the filament and the mandrel. Such strains and twists appear to be inherent in this method of operation and do not seriously affect filament quality except in the final (second or third) coiling operations where the distortion is of greater magnitude.

Conventional heat treating consists in passing the filament and mandrel combination through a furnace at a speed which provides the desired treatment and may also consist of other treat-

ments in which lengths of said filament and mandrel combination equivalent to several filaments (ten for instance) are placed in a boat in a furnace for the desired length of time. In such treatments the mandrels must be left in the coils of the filament wire to keep them in position and therefore must be considered in the heat treatment. The final mandrel in multiple coil filaments is of considerable size and, because of its mass and position within an irregular filament, is effective in changing the rate and uniformity of heating and cooling. The final mandrel is also of a different material than the filament and is apt to contaminate said filament during heat treatment. To remove all the mandrels from the filament coils before heat treatment is impractical because of the large amount of unwinding and distortion taking place. These heat treatments take a relatively long time in comparison to my method and, when the filaments are piled one on the other, are objectionable because of the pressure and restraining effect of the filaments on each other.

My process on the other hand is particularly well suited to produce more stable and uniform filaments and permits manufacture of filaments having more desirably shaped end sections than possible before. The uniformity appears as an increase in consistency in the number of coils and the length of wire turn by turn (i. e. equal weight) of the filaments.

According to my invention the filament wire, which is preferably of the so-called non-sag variety, is first coiled about a comparatively long mandrel preferably at a uniform pitch and, if the filament is to be of the triple helical type, is again coiled with the mandrel about a second mandrel. Both these operations are performed in the usual manner and result in the filament wire taking a given shape and developing strains and a tendency to straighten out an appreciable amount. Accordingly the filament and mandrel assembly are heat treated in the conventional way to remove a considerable portion of the said strains and the tendency to unwind. From this mandrel and filament coil assembly individual coiled-coil or triple coiled filaments are made one after another successively. The operations in the manufacture of coiled coil filaments are, first, to lay a portion of the mandrel and filament coil assembly parallel to a second temporary mandrel, to coil a succeeding portion of said assembly about said temporary mandrel at a given pitch, to draw out a still further succeeding portion of said assembly beyond the end of the temporary

mandrel, to sever the second straight portion of the assembly and then to withdraw said temporary mandrel. In the manufacture of triple coiled filaments the operations are the same except that an assembly including the twice coiled filament wire and both the first and second mandrels is coiled on the temporary mandrel which is then the third mandrel. The end portions of the filaments form legs which lie parallel to the axis of the filament and which are therefore well adapted to be attached to the leading-in wires of a lamp. This shape of leg cannot be produced by the conventional methods of manufacture. The limited time of the coiling operation prevents coiling strains from building up to a point where they are detrimental and allows the recoil to loosen the whole filament coil on the mandrel so that it can be withdrawn. The recoil is affected by physical characteristics of the mandrel used in the first coil and also alteration of these characteristics in subsequent heat treatment of both the filament coil and mandrel assembly. The individual filaments are then heat treated to cause them to be set in the coiled coil or triple coiled form whereupon the other fixed mandrels are removed, preferably by dissolving in acid. The filaments are then mounted on the leading-in wires of incandescent lamps which are finally completed by being operated at normal and abnormal rates for short intervals. The primary factor in the success of my process is believed to be the operations including the first heat treatment, the winding of the mandrel and filament wire assembly on the final (temporary) mandrel and the removal of said final or temporary mandrel before further work (heat treatment) is done on the filament wire.

The advantages of my process of manufacture will be more readily understood from the detailed description which follows of one specific application of my process and from the drawing.

The drawing illustrates diagrammatically in Figs. 1 to 7 inclusive the various steps in the process of my invention.

To show specifically all features of the process of my invention, I will hereinafter describe my preferred method of manufacturing the double helical or coiled coil filament for a 115 volt, 60 watt incandescent lamp. The tungsten filament wire 10 of 1.85 mils diameter is shown in Fig. 1. This wire 10 is preferably of the type having non-sag characteristics or such as to develop said characteristics before the lamp is burned any appreciable time and may be either of the cleaned or the uncleaned variety. If non-sag, the wire 10 is preferably made according to the Pacz Patent 1,410,499 of March 21, 1922. Uncleaned wire is that still retaining the coating formed by the graphite, etc., lubricant used in the drawing process. Because of the lubricating value of the coating in coiling the wire, and the expense of removing it, said coating is preferably left thereon.

The filament wire 10 is coiled about a wire mandrel 11 as shown in Fig. 2, said mandrel 11 being four mils in diameter and of sufficient length to be conveniently spooled. The filament wire 10 in this instance is coiled at a pitch of 335 turns per inch on a mandrel 11 which is preferably made of molybdenum or some other material of which there is a minimum danger of melting or of contaminating said filament in the heat treating operation and which can be easily removed therefrom. If the filament is of the triple helical type, the filament wire and mandrel assembly are again

coiled on a second mandrel before passing to the next manufacturing step.

The mandrel and filament wire assembly 12 is now subjected to a heat treatment, as shown in Fig. 3, designed to remove a considerable portion of the original drawn mandrel and original drawn filament wire strains as well as later coiling strains therein and to partially clean it. The treatment is preferably divided into two sections, the first being for about twelve seconds when the mandrel and the filament wire assembly 12 is passed through a furnace 13 containing wet or humidified hydrogen and retained at 1400° C., and the second being for about sixteen seconds when said assembly 12 is passed through a second furnace 13 containing substantially dry (dehydrated) hydrogen and retained at 1500° to 1700° C. The furnace 13 illustrated is provided with an electrical heating element 14. In the first section of the treatment, the moisture in the hydrogen combines with the graphite of the coating to partially clean the filament wire and mandrel assembly 12 and the heat promotes this action as well as removes a portion of the strains. In the second section of the treatment the heat removes a considerable portion of the strains in the filament assembly 12. Both sections of the treatment are not always required in which case only the second section thereof is used. This is particularly true when the cleaned filament wire 12 is used although for the uncleaned wire wet hydrogen is preferred. Dry hydrogen can be used in both heat treatments if desired.

After the heat treatment the mandrel and filament wire assembly 12 is coiled on a second temporary mandrel 15, as shown in Fig. 4. This mandrel 15 is the third mandrel when triple coiled filaments are being formed. The operation is preferably performed by a machine of the type shown in Illingworth Patent No. 1,771,927 of July 29, 1930, and is an intermittent operation interrupted at intervals while straight end portions of the filament are produced and while the completed filament is severed from the remainder. As shown, one end of the mandrel and filament wire assembly 12 is first gripped between the jaws 16 and 17 whereupon the spindle 18 carrying the mandrel and filament wire assembly 12 is rotated about the axis of the second mandrel 15 as said mandrel 15 and jaws 16 and 17 are moved at the desired rate away from the spindle 18. The mandrel and filament wire assembly 12 passes through an off-center hole in the spindle 18 and is wound around the temporary mandrel 15 by the rotation of said spindle 18. The movement of the mandrel 15 and the jaws 16 and 17 away from the spindle 18 causes the windings to be advanced along the mandrel 15. In this instance the jaws 16 and 17 hold 168 mils (4 mm.) of the mandrel and filament wire assembly 12, and the mandrel 15 is approximately 15.3 mils in diameter. The coiling is done at a pitch of 76 turns per inch but only 41 turns are placed on the mandrel 15 before the end of the mandrel is reached and rotation of the spindle 18 is stopped. A straight section 19 (Fig. 5) substantially the equivalent of two of the 168 mil end portions is now drawn out whereupon all motion stops.

An individual coiled coil filament in the instance illustrated is now completely formed and, as shown in Fig. 5, the straight portion 19 is severed by the knives 20 and 21. The knives 20 and 21 are so positioned with respect to the coiled coil portion of the filament as to leave on that end a straight leg 168 mils in length, the equiv-

5 alent of the straight leg at the other end of said portion. The legs are both parallel to the longitudinal axis of the filament and can now be bent to some other angle if desired. The temporary mandrel 15 is then moved to the left to withdraw it from the filament and jaw 16 whereupon the jaws 16 and 17 are separated, thereby freeing the filament 22 and allowing it to drop out of position. A new filament is started by movement 10 of jaws 16 and 17 toward the spindle 18 which places the new end of the mandrel and filament wire assembly 12 between the said jaws 16 and 17. The mandrel 15 is also moved to the right and enters the aperture in the spindle 18 before the coiling operation begins. The filaments released from the machine are very uniform in 15 length, have equal straight legs at both ends parallel to the axis of the coiled coil portion and have expanded so that the latter coils now have a pitch of 69 turns per inch. The unwinding of the latter coils is not of serious consequence as it has occurred evenly from end to end. When the final, or temporary mandrel in this case, is not removed, as in the conventional method 20 of operation, only the end portions unwind and the coils are set in this position in the heat treatment. The unwinding of the filament wire on the fixed mandrel is negligible since it effects such a very small portion of the total amount of filament wire.

30 The filaments 22 are heat treated again, this time to set the coiled coil or triple coiled portion, as the case may be, and to remove further strains. The treatment, as shown in Fig. 6, preferably takes place in apparatus which treats said filaments individually and which is the subject matter of my co-pending application Serial No. 133,854, filed March 30, 1937. In this apparatus the filaments are placed in a tungsten boat 23 of exceedingly small mass and are inserted in the resistance coil 24 of the furnace 25. The coil 24 in this instance is heated to 2000-2200° C. by the passage of electricity therethrough and heats the filament 22 and boat 23 which are removed therefrom after 5 seconds. Tungsten is the material preferred for the boat since it cannot contaminate the filament and withstand the high temperatures of the treatment. A steady influx 40 of a non-oxidizing gas, in this case substantially dry hydrogen, is introduced into the furnace 25 through the pipe 26 to prevent oxidation of the filament 22, the resistance coil 24, the boat 23 and other parts heated by the said coil 24. It is presumed that a portion of the total time of the treatment is taken to bring the filament 22 to the maximum temperature thereof because of the small mass of the boat 23 and its proximity to the heating coil 24. Upon being withdrawn from the resistance coil 24, one second is allowed for the filament 22 to cool whereupon it is removed from the furnace 25.

45 With different sizes and kinds of filament wire it is desirable to change the treatment accordingly and generally a treatment for between three and five seconds in a furnace at a temperature between 1900 and 2300° C. is sufficient for most filaments of the smaller conventional sizes. The temperature of the treatment is selected from the behavior of the filament which becomes brittle if too high a temperature is used and is not sufficiently relieved of its strains if the temperature is too low. The optimum temperature is a compromise and is considered to be that which produces the most satisfactory filament both for performance and for commercial lamp production

5 methods. The temperatures indicated were measured by an optical pyrometer sighted through a window in the furnace wall and onto the resistance coil 24 and have been found to be about 225° C. higher than that reached by the boat 23 and the filament 22 and the truest obtainable. In measuring the temperature of the resistance coil 24, the readings are corrected for the transmission factor of the window. Difficulty is experienced in making absolute temperature 10 measurements because of the high emissivity of the tungsten coil 24, tungsten boat 23 and filament assembly 12 which leads to considerable error in apparent temperature readings in comparison to black body conditions. The 225° difference in temperature between the resistance coil 24 and the filament 22 was found by experiments in which quantities of highly purified platinum and  $Al_2O_3$  were melted in the boat 23. Platinum and  $Al_2O_3$  melt at 1755° C. and 2050° C. 20 respectively and where caused to melt in the boat 23 during the regular treating procedure when the resistance coil 24 was at 1980° C. and 2275° C. respectively. These substances were placed in the boat 23 with and without the filament assembly 12 and outside and inside the said assembly 12 and only slightly different temperatures were required to cause melting in each case. It appears that the 60 watt filament assembly is only heated to between 1725 and 1875° C. when the 30 resistance coil is at between 2000 and 2200° C. If larger and more special types of filaments are treated slightly higher temperatures are often required and the treatment is lengthened to as much as 30 seconds.

35 The wattage of electricity consumed by the resistance coil is used to indicate the temperature of the treatment after the initial temperature readings are taken. During the heat treatment the filament 22 contracts slightly so that the final coils are now at substantially 69½ turns per inch. This change in filament length has been found to vary considerably in the acceptable range of the heat treatment and it has been found possible to alter the length of the filament somewhat by 40 changing the temperature of the treatment. Higher temperatures cause a greater increase in the length of the filament.

45 The fixed mandrel 11, or both fixed mandrels as the case may be, are now removed whereupon the filament 22 is mounted on the inner structure of the lamp. The mandrel 11 is preferably removed chemically by dissolving it in acid whereupon the filament 22 is rinsed and dried in the usual way. During this operation the filament contracts until the pitch is 70 turns per inch which shows that not all of the strains are removed in the particular instance by the heat treatments. Photomicrographs of the filament at this point show that very little if any change has occurred in the wire during heat treatment since it is still fibrous. The structure of the molybdenum mandrel on the other hand is no longer fibrous but indicates considerable development of grain size approaching that of single crystals.

55 The filaments 22 being either of coiled coil or triple coiled construction are very concentrated and, being treated according to my method, are simply mounted on the lead-in wires 27 and 28 of the lamp shown in Fig. 7 and are preferably 60 engaged by one intermediate support 29. The straight singly coiled legs of the filament 22 are clamped in hooks at the ends of the leading-in wires 27 and 28 which are designed to hold said filament 22 when cold under slight tension to 75

facilitate uniform mounting. After mounting, the filament 22 is found to have 60 turns per inch in the final coils.

The lamp is now completely assembled whereupon the filament 22 is permanently set and whatever getter is introduced thereon is driven off by operating the lamp at normal and abnormal voltages for very short intervals of time. During this process the filament again changes shape slightly and in quantity production the second coiling is found to have a pitch of between 58 and 62 turns per inch. This range of difference is acceptable for commercial lamp production since the changes in the filaments are more general than before and are consequently of much less importance. Obviously there is no means for calculating the amount of change which takes place in the filament 22 during the manufacture of the lamp, but I have found that once the desired final conditions are reached by trial, my process assures that these same results are secured regularly within a practical range.

What I claim as new and desire to secure by Letters Patent of the United States is:

- 25 1. The process of making multiple coil filaments which consists in winding a filament wire around a mandrel; heat treating the mandrel and the filament wire assembly to remove a considerable part of the strains therein produced chiefly by the coiling operation; coiling the mandrel and the filament wire assembly about a second temporary mandrel; withdrawing the second temporary mandrel before further heat treatment and immediately heat treating the first mandrel and the filament wire assembly a second time to remove a considerable part of the strains therein resulting from the second coiling operation and to set the filament; and removing the first mandrel from the filament coil.
- 30 2. The process of making multiple coil filaments which consists in winding a filament wire around a mandrel; heat treating the mandrel and the filament wire assembly to remove a considerable part of the strains therein produced chiefly by the coiling operation; repeatedly coiling a portion of the mandrel and the filament wire assembly about a second temporary mandrel, severing it to form individual coiled coil filaments, and immediately withdrawing the second temporary mandrel before further heat treatment; then heat treating said filaments to set them and finally removing the first mandrel from the said individual filaments.
- 35 3. The process of making multiple coil filaments which consists in winding a filament wire around a mandrel; heat treating the mandrel and the filament wire assembly to remove a considerable part of the strains therein produced chiefly by the coiling operation; repeatedly coiling a portion of the mandrel and the filament wire assembly about a second temporary mandrel, severing it to form individual coiled coil filaments and immediately withdrawing the second temporary mandrel before further heat treatment; heat treating each of the said individual filaments separately to remove a considerable part of the strains therein resulting from the second coiling operation and to set the filaments; and removing the first mandrel from the said individual filaments.
- 40 4. The process of making multiple coil filaments which consists in winding a filament wire around a mandrel; heat treating the mandrel and the filament wire assembly to remove a considerable part of the strains therein produced chiefly by the coiling operation; forming from said mandrel and filament assembly a plurality of individual coiled coil filaments with straight end portions by winding the intermediate portion around a second temporary mandrel and severing the one end portion from the remainder of said assembly, immediately withdrawing said second temporary mandrel before further heat treatment; heat treating the filaments to remove a considerable amount of the strains produced by the second coiling and to set the filaments; and removing the first mandrel from said filaments.
- 45 5. The process of making multiple coil tungsten filaments which consists in winding a filament wire around a mandrel; heat treating the mandrel and the filament wire assembly to remove a considerable part of the strains therein produced chiefly by the coiling operation; coiling the mandrel and the filament wire assembly about a second temporary mandrel and immediately withdrawing the second temporary mandrel before further heat treatment; heating the first mandrel and the filament wire assembly to a temperature of approximately 1675 to 2075° C. for from three to five seconds in a non-oxidizing atmosphere to remove a considerable portion of the strains therein resulting from the second coiling operation and to set the filament; and removing the first mandrel from the filament coil.
- 50 6. The process of making multiple coil tungsten filaments which consists in winding a filament wire around a mandrel; heat treating the mandrel and the filament wire assembly to remove a considerable part of the strains therein produced chiefly by the coiling operation; coiling the mandrel and the filament wire assembly about a second temporary mandrel and immediately withdrawing the second temporary mandrel before further heat treatment; heating the first mandrel and the filament wire assembly to a temperature of approximately 1775 to 1975° C. for about five seconds in a non-oxidizing atmosphere to remove a considerable portion of the strains therein resulting from the second coiling operation and to set the filament; and removing the first mandrel from the filament coil.
- 55 7. The process of making multiple coil tungsten filaments which consists in winding a filament wire around a mandrel; heating the mandrel and the filament wire assembly to approximately 1500 to 1700° C. for about sixteen seconds in a non-oxidizing atmosphere to remove a considerable part of the strains therein produced chiefly by the coiling operation; coiling the mandrel and the filament wire assembly about a second temporary mandrel and immediately withdrawing the second temporary mandrel before further heat treatment; heating the first mandrel and the filament wire assembly to a temperature of approximately 1675 to 2075° C. for from three to five seconds in a non-oxidizing atmosphere to remove a considerable portion of the strains therein produced by the second coiling operation and to set the filament; and removing the first mandrel from the filament coil.
- 60 8. The process of making multiple coil tungsten filaments which consists in winding a filament wire about a mandrel; heating the mandrel and the filament wire assembly to approximately 1500 to 1700° C. for about sixteen seconds in a non-oxidizing atmosphere to remove a considerable part of the strains therein produced by the coiling operation; repeatedly coiling a portion of the mandrel and the filament wire assembly about

5 a second temporary mandrel, severing it to form individual coiled coil filaments and immediately withdrawing the second temporary mandrel before further heat treatment; heating the individual coiled coil filaments to approximately 1775 to 1975° C. for about five seconds in a non-oxidizing atmosphere to remove a considerable portion of the strains therein resulting from the second coiling operation and to set the filaments; 10 and removing the first mandrel from the filaments.

15 9. The process of making multiple coil tungsten filaments which consists in winding a filament wire about a mandrel; winding the mandrel and the filament assembly about a second mandrel; heating the mandrel and the filament wire assembly to approximately 1500 to 1700° C. for

about sixteen seconds in a non-oxidizing atmosphere to remove a considerable part of the strains therein produced chiefly by the coiling operation; repeatedly coiling the mandrel and the filament wire assembly about a third temporary mandrel, 5 severing it to form individual triple coiled filaments, and immediately withdrawing the third temporary mandrel before further heat treatment, heating the triple coiled filament assembly to approximately 1775 to 1975° C. for about 10 five seconds in a non-oxidizing atmosphere to remove a considerable portion of the strains therein produced by the third coiling operation and to set the filament; and removing the first and second mandrels from said filaments. 15

WILLIAM P. ZABEL.

CERTIFICATE OF CORRECTION.

Patent No. 2,142,865.

January 3, 1939.

WILLIAM P. ZABEL.

It is hereby certified that error appears in the printed specification of the above numbered patent requiring correction as follows: Page 4, first column, line 32, claim 1, after "mandrel" strike out the semicolon and insert instead the words and immediately; line 34, same claim, strike out "and immediately" and insert instead a semicolon; and that the said Letters Patent should be read with this correction therein that the same may conform to the record of the case in the Patent Office.

Signed and sealed this 21st day of February, A. D. 1939.

(Seal)

Henry Van Arsdale.  
Acting Commissioner of Patents.

5 a second temporary mandrel, severing it to form individual coiled coil filaments and immediately withdrawing the second temporary mandrel before further heat treatment; heating the individual coiled coil filaments to approximately 1775 to 1975° C. for about five seconds in a non-oxidizing atmosphere to remove a considerable portion of the strains therein resulting from the second coiling operation and to set the filaments; 10 and removing the first mandrel from the filaments.

15 9. The process of making multiple coil tungsten filaments which consists in winding a filament wire about a mandrel; winding the mandrel and the filament assembly about a second mandrel; heating the mandrel and the filament wire assembly to approximately 1500 to 1700° C. for

about sixteen seconds in a non-oxidizing atmosphere to remove a considerable part of the strains therein produced chiefly by the coiling operation; repeatedly coiling the mandrel and the filament wire assembly about a third temporary mandrel, 5 severing it to form individual triple coiled filaments, and immediately withdrawing the third temporary mandrel before further heat treatment, heating the triple coiled filament assembly to approximately 1775 to 1975° C. for about 10 five seconds in a non-oxidizing atmosphere to remove a considerable portion of the strains therein produced by the third coiling operation and to set the filament; and removing the first and second mandrels from said filaments. 15

WILLIAM P. ZABEL.

CERTIFICATE OF CORRECTION.

Patent No. 2,142,865.

January 3, 1939.

WILLIAM P. ZABEL.

It is hereby certified that error appears in the printed specification of the above numbered patent requiring correction as follows: Page 4, first column, line 32, claim 1, after "mandrel" strike out the semicolon and insert instead the words and immediately; line 34, same claim, strike out "and immediately" and insert instead a semicolon; and that the said Letters Patent should be read with this correction therein that the same may conform to the record of the case in the Patent Office.

Signed and sealed this 21st day of February, A. D. 1939.

(Seal)

Henry Van Arsdale.  
Acting Commissioner of Patents.